

May 21, 1968

R. R. HALIK ET AL

3,384,574

CATALYTIC PROCESS FOR MAKING A JET FUEL

Filed July 21, 1966

4 Sheets-Sheet 1

HEATING VALUE Vs. PARAFFIN CONTENT OF JET FUELS



FIG. I

Inventors  
Raymond R. Halik  
Fritz A. Smith  
Carl W. Streed  
Henry R. Ireland

By *Carl W. Streed*  
Agent

May 21, 1968

R. R. HALIK ET AL

3,384,574

CATALYTIC PROCESS FOR MAKING A JET FUEL

Filed July 21, 1966

4 Sheets-Sheet 2

LUMINOMETER NUMBER Vs. PARAFFIN CONTENT



FIG. II

*Inventors*

Raymond R. Halik  
Fritz A. Smith  
Carl W. Steed  
Henry R. Ireland

By *Carl W. Steed*  
Agent

May 21, 1968

R. R. HALIK ET AL

3,384,574

CATALYTIC PROCESS FOR MAKING A JET FUEL

Filed July 21, 1966

4 Sheets-Sheet 3

RELATIONSHIP BETWEEN EQUILIBRIUM AROMATIC- NAPHTHENE  
RATIOS, PRESSURE AND TEMPERATURE



FIG. III

Inventors

Raymond R. Halik  
Fritz A. Smith  
Carl W. Streed  
Henry R. Ireland

By *Paul M. Farnsworth*  
Agent

May 21, 1968

R. R. HALIK ET AL

3,384,574

CATALYTIC PROCESS FOR MAKING A JET FUEL

Filed July 21, 1966

4 Sheets-Sheet 4

ESTIMATION OF JET FUEL FREEZE POINT FROM 370° F WEST TEXAS DATA



FIG. IV

Inventors  
Raymond R. Halik  
Fritz A. Smith  
Carl W. Streed  
Henry R. Ireland

By *Carl W. Streed*

Agent

## 1

3,384,574  
CATALYTIC PROCESS FOR MAKING  
A JET FUEL

Raymond R. Halik, Pitman, Henry R. Ireland, West Deptford Township, Gloucester County, Fritz A. Smith, Cherry Hill, and Carl W. Streed, Haddonfield, N.J., assignors to Mobil Oil Corporation, a corporation of New York

Continuation-in-part of application Ser. No. 478,526, July 27, 1965. This application July 21, 1966, Ser. No. 567,007

6 Claims. (Cl. 208—138)

### ABSTRACT OF THE DISCLOSURE

The disclosure is concerned with the method of producing jet fuels from predetermined correlations represented by FIGURES I through IV in which the method includes determining from the correlation of FIGURE IV the permissible n-paraffin content of a desired freeze point jet fuel product, determining from FIGURES I and II the maximum naphthalene to aromatic ratio tolerable in a product of desired heating value and luminometer number, and catalytically reforming a paraffin containing kerosine feed in accordance with the relationship represented by FIGURE III for the above predetermined naphthalene/aromatic ratio under space velocity conditions to permit 70% retention of paraffins.

This application is a continuation-in-part of application Ser. No. 478,526 filed July 27, 1965, now abandoned entitled "Catalytic Process and Novel Compositions Prepared Therefrom." The present invention relates to an improved method and process for the preparation of hydrocarbon fuel compositions of desired heating value suitable for use in gas turbine engines.

In a more particular aspect, the invention relates to the method and combination of process steps for preparing from petroleum distillate fractions, high quality jet fuels under conditions to preserve paraffinic components of the distillate fractions. More specifically, the invention relates to defining a method for converting relatively high boiling hydrocarbon feed stock materials boiling in the range of kerosine type jet fuel to product rich in paraffins providing product specification luminometer number, freeze point and desired heating value.

In accordance with the method of this invention, desired paraffin rich jet fuels are prepared from petroleum hydrocarbon fractions of the kerosine type composed substantially of hydrocarbon mixtures boiling in the range of from about 350 up to about 550° F. and preferably boiling in the range of from about 375° F. up to about 525° F. Suitable hydrocarbon feeds include paraffin rich fractions boiling within the above-identified range and include virgin kerosines having an ASTM boiling range of from about 375 to about 525° F. derived from a variety of crude sources including Mid-Continent, Barco, West Texas, and Middle East (Kuwait) crudes. The feed stocks employed in the method herein described comprise kerosine type fractions containing paraffins, naphthalenes and aromatics in amounts of from about 30 to about 75 weight percent paraffins, from about 20 to about 50 weight percent naphthalenes, and from about 5 to about 30 weight percent aromatics. Particularly desirable feed materials that may be

## 2

upgraded by the method of this invention include straight run kerosine fractions of the following composition.

|              | Mid-Continent |      | Barco |      | W. Texas |      |
|--------------|---------------|------|-------|------|----------|------|
|              | Wt.           | Vol. | Wt.   | Vol. | Wt.      | Vol. |
| Paraffins    | 39.9          | 42.7 | 42.4  | 45.1 | 58.6     | 61.0 |
| Naphthalenes | 43.1          | 42.1 | 43.3  | 42.0 | 33.2     | 31.8 |
| Aromatics    | 17.0          | 15.2 | 14.3  | 12.9 | 8.2      | 7.1  |

In accordance with the method of this invention, a kerosine boiling hydrocarbon fraction is subjected to a catalytic reforming treatment comprising primarily catalytic dehydrogenation and isomerization reactions under conditions selected to convert naphthalenes to aromatics and hydroisomerize n-paraffins in the feed fraction under conditions directed to reduce any significant reduction of paraffins in the feed. Thereafter substantially complete removal of aromatics materials in the product of the catalytically treated mixture is effected by SO<sub>2</sub> extraction or other convenient methods to produce a desired low concentration of aromatic in the high quality jet fuel.

In the event that the relatively high boiling feed stocks employed in the method of this invention contains materials or impurities considered deleterious to the catalyst used in the catalytic reforming treatment above referred to, the feed stocks are subjected to a pretreatment for removal or substantial reduction in concentration of such impurities. That is, feed stocks that contain a relatively high concentration of sulfur as an impurity are pretreated to reduce the sulfur concentration below about 100 p.p.m. and preferably below about 40 p.p.m. and more usually less than about 20 parts/million. It is also desirable to effect substantially complete removal of other undesirable impurities, such as arsenic and lead in one or more pretreatment steps. In particular, when the feed stocks contain a concentration of nitrogen substantially in excess of 20 parts/million, the feed stock is pretreated to substantially reduce the nitrogen concentration thereof to a low value which is usually less than about 20 parts/million (p.p.m.) and preferably is less than about 10 parts/million. For example, a virgin kerosine fraction boiling in the range of 375–500° F. and obtained from a Mid-Continent crude may contain a concentration of sulfur up to about 1700 p.p.m.; a virgin kerosine fraction of about the same boiling range obtained from Barco crude may contain up to about 700 p.p.m.; and a similar boiling range kerosine fraction obtained from a West Texas crude may contain up to about 350 p.p.m. sulfur. These feed materials are therefore subjected to a suitable desulfurizing pretreatment to reduce the sulfur and any nitrogen constituents therein to not more than about 20 p.p.m. and preferably less than 20 p.p.m. To accomplish this pretreatment the feed stock is subjected to hydrodesulfurization and hydrodenitrogenation conditions by contact with a suitable catalyst (e.g., cobalt molybdate on alumina, nickel-tungsten sulfide, chromia on alumina, and others) known in the art in the presence of hydrogen at conditions of pressure, space velocity and temperature to reduce the concentration of sulfur and nitrogen to desired values. Arsenic and lead would be simultaneously removed in such a hydropretreatment but may be separately removed by simple contact with porous alumina at reforming temperature conditions. Pretreatment of the feed stocks to remove sulfur and nitrogen compounds therefrom may be accomplished particularly by contact with a cobalt molybdate hydropretreat-

ment catalyst within the following ranges of operating conditions.

Space velocity (LHSV) ..... 0.5-10  
 Hydrogen partial pressure (p.s.i.g.) ..... 130-800  
 Temperature, ° F. ..... 675-800  
 Hydrogen circulation rate (s.c.f./bbl.) ..... 190-3000

The kerosine boiling feed stock thus treated and substantially freed of undesired impurities is then subjected to the catalytic reforming treatment of this invention under conditions correlated as hereinafter described in the presence of a suitable dehydrogenation-isomerizing catalyst such that, the reactions effected will maintain a relatively high percentage of the feed paraffins, and in certain instances increase the paraffinic concentration thereof. That is, it has been found that by correlating operating conditions as described more fully hereinafter that the relatively high boiling feed stocks can be catalytically reformed to provide a product mixture composed of hydrocarbons boiling substantially in the same range as the feed stock having a markedly reduced concentration of naphthenes while retaining a relatively high concentration of feed paraffins. It appears from the data obtained in this investigation that the main reaction is primarily dehydrogenation of naphthenes and such dehydrogenation may be made to occur in the substantial absence of paraffin cracking to substances that boil lower than the feed stock. However, even if some limited cracking of paraffins occurs, the operating conditions employed are such that the paraffinic concentration is none-the-less maintained at a very high level, possibly due to the conversion of some ring compounds in the feed stock to paraffins of corresponding carbon atoms content which boil in the range of the feed stock. Accordingly, the feed stocks employed herein are subjected to controlled catalytic dehydrogenation and catalytic isomerization under selected operating conditions that substantially completely and unexpectedly conserve the paraffinic concentration of the feed while substantially decreasing the naphthene concentration therein to aromatics. A desired paraffin rich jet fuel product fraction is obtained therefrom by removal of aromatics from the product.

Reference is made above to conservation or retention of the paraffinic concentration of the feed stock. By this we intended to include within the broad aspect thereof some variance from the paraffinic concentration of the feed stock, the extent of variance being dependent on factors including the particular combination of conditions used for the catalytic reforming treatment, the desired freeze point requirements of the jet fuel to be produced, the particular feed stock employed, and other characteristics. Hence, it is not intended to exclude production of catalytically treated mixtures having less than 70% retention of the paraffinic concentration of the feed stock, as the production of such catalytically treated mixtures is within the scope of this invention even though it is preferred to operate under conditions which produce no significant loss in the paraffin constituent of the feed. The invention is generally carried out under conditions to the extent of producing catalytically reformed product mixtures that retain a paraffinic concentration of at least about 70% of the paraffinic concentration of the feed stock and in most cases preferably retain more than about 80% of the paraffinic concentration of the feed stock.

Catalysts suitable for use in the reforming operation herein described include the metals of the platinum series on a suitable carrier material such as alumina. Generally, the catalyst employed should be a dehydrogenation catalyst of the platinum type having relatively little or a low cracking activity but possessing isomerizing activity at selected operating conditions. Accordingly, the catalyst may be one comprising from about 0.1 up to about 1.0 percent platinum on alumina (e.g., eta alumina) or a low activity silica-alumina base. The catalyst may also contain a halogen promotor such as chlorine or fluorine in

an amount of up to about 2.0% and, preferably, in an amount less than about 1%. In a more particular aspect, the reforming catalysts contain from about 0.3 to about 0.8% platinum. However, also suitable for use herein are those catalysts which are known to possess activity for dehydrogenating naphthenes to aromatics and having a relatively low cracking activity. Examples of such catalysts include tungsten and/or nickel on kieselguhr, chromium oxide on alumina, and others.

Although the reforming conditions comprising dehydrogenation of naphthenes to aromatics and isomerization of paraffins can be varied, depending on the composition of the feed stock employed and the desired properties of the jet fuel product; the conditions of operation are correlated within the following general ranges of conditions as discussed more fully hereinafter.

|                                   | Broad        | Preferred    |
|-----------------------------------|--------------|--------------|
| Space Velocity (LHSV)             | 0.5-60       | 1-20         |
| H <sub>2</sub> /feed, s.c.f./bbl. | 2,000-15,000 | 4,000-10,000 |
| Average Temperature, ° F.         | 640-980      | 780-900      |
| Hydrogen Pressure, p.s.i.         | 20-1,400     | 100-500      |

That is, when it is desired to obtain a desired naphthene dehydrogenation without regard to effecting any significant degree of isomerization of the normal paraffins in the feed fraction, reforming of the kerosine boiling feed may be effected within the following operating conditions.

At an average temperature of at least about 800° F., a space velocity (LHSV) of at least 0.5 is employed. At an average temperature of at least about 850° F., a space velocity (LHSV) of more than 3 is employed. At an average temperature of at least about 900° F., a space velocity (LHSV) of at least 10 is employed. At an average temperature of at least about 940° F., a space velocity (LHSV) of more than 20 is employed. As described more fully hereinafter, the preferred pressure of operation is also a function of operating temperature, as well as a function of the degree of naphthene dehydrogenation desired. The greater the degree of dehydrogenation and/or the lower the temperature, the lower the maximum permissible pressure.

On the other hand, when obtaining the desired naphthene dehydrogenation, while simultaneously effecting the substantial isomerization of normal paraffins in the feed fraction, in a single stage of contact of the feed with a bed of catalyst, the following conditions are preferably employed.

Average temperature ..... ° F. > about 875  
 Space velocity (LHSV) ..... > 5  
 Total pressure ..... p.s.i.g. > 500

In one embodiment of this invention, the process comprises the catalytic treatment of the relatively high boiling kerosine feed stocks in a combination of steps comprising desulfurization of the feed followed by catalytic reforming of the desulfurized feed in at least two stages wherein, in a first reforming stage, the feed stock is processed under conditions to effect primarily naphthene dehydrogenation and in a second reforming stage, conditions promoting isomerization of paraffin constituents are selected. Under some isomerizing conditions dehydrogenation of naphthenes can also be expected in the second step in a minor amount and generally is only a small fraction of that obtained in the first reforming stage. The method and process conditions selected for dehydrogenating and isomerizing as described herein can be effected in at least two or more catalytic beds in a single reactor, or the reactions may be accomplished substantially separately in a plurality of sequentially arranged reactors. Furthermore, suitable heat exchange means for heating or cooling may be provided for adjusting the temperature of the hydrocarbon reactants between catalyst beds or between reactor zones. However, in any arrangement selected, it is important that the catalyst be arranged to

obtained temperature profiles and space velocities suitable for maintaining the desired stages of chemical conversion comprising primarily dehydrogenation in one first stage of catalyst contact and primarily isomerization in a downstream catalyst contact step comprising the same or a separate bed of catalyst. To optimize naphthene dehydrogenation and effect substantial isomerization of n-paraffins, while conserving the paraffin content of the feed stock, the embodiment above discussed is preferably carried out under the following conditions for the first and second stages of catalyst contact.

#### FIRST STAGE

Temperature ----- At least about 825° F. but not more than about 925° F. as the inlet temperature of the feed. 10  
 Space velocity ----- More than 5 (LHSV).  
 Pressure (total) ----- Below 500 p.s.i.g.  
 Catalyst ----- As described hereinbefore, e.g., platinum or alumina, with or without chlorine but when present, preferably not more than 1% chlorine. 20

#### SECOND STAGE

Space velocity ----- Below 5 (LHSV).  
 Total pressure ----- Below 500 p.s.i.g.  
 Inlet temperature ----- Generally not substantially over 850° F. and at temperatures minimizing cracking under the isomerizing conditions. 30  
 Outlet temperature ----- At least 750° F.  
 Catalyst ----- E.g., platinum on alumina containing preferably not more than 1% chlorine.

Depending upon the freeze point requirements of the ultimately produced jet fuel product, the method herein described can be carried out to process feed fractions that comprise a kerosine fraction as aforescribed blended with alkylate in blends containing up to about 40% or more by weight of alkylate. Generally speaking, and by use of a blend containing from about 25 to about 40% by weight of alkylate, sufficient isoparaffins may be generally present in the feed blend whereby products of sufficiently low freeze point can be obtained by subjecting the feed blend to a single stage of catalytic reforming comprising primarily naphthene-dehydrogenation conditions without need to also effect isomerization of n-paraffins present in the kerosine portion of the feed blend. On the other hand, with feeds that comprise the aforescribed kerosine fractions per se or blends thereof with, for example, less than 25% by weight of alkylate, it may be desirable to not only effect naphthene dehydrogenation but, also, substantial isomerization of n-paraffins in the kerosine portion in order to provide end products of exceptionally low and desired freeze point characteristics. Therefore, when processing low alkylate-containing blends, the process conditions may be controlled more carefully in a multi-stage catalyst bed system when it is desired to produce low freeze point products.

On the other hand, when processing a feed that comprises a kerosine fraction blended with an alkylate fraction, the alkylate fraction that is employed will have a boiling range that falls substantially within the boiling range of the kerosine fraction. It can, for purposes of illustration, be an alkylate composed substantially within the boiling range of the kerosine fraction. It can, for purposes of illustration, be an alkylate composed substantially of isoparaffins, or such alklates that contain a minor amount (e.g., 5-15%) naphthenes and/or small amounts of olefins (e.g., 1-3%). When alkylates of the latter type are used, and particularly if they also contain impurities such as sulfur and/or nitrogen, the impurities are removed sufficiently by pretreatment (e.g., hydrodesulfurization) of the alkylate feed or feed blend as discussed

above prior to subjecting the feed to the naphthene-dehydrogenation reactions described herein.

Thus, in the use of blends of the kerosine fraction and alkylate, and in cases wherein the combination of the feed components is deficient in isoparaffin content (e.g., in such blends containing below 25% of alkylate), end products of exceptionally low freeze points are obtained by subjecting the feed blend preferably to two-stage of catalytic treatment under the following conditions.

#### FIRST STAGE

Temperature ----- At least 800° F., but not more than about 860° F. as the inlet temperature of the feed. 10  
 Space velocity ----- More than 5 (LHSV).  
 Pressure (total) ----- Below 500 p.s.i.g.  
 Catalyst ----- As described hereinbefore, e.g., platinum on alumina, with or without chlorine but, when present, preferably not more than 1% chlorine. 20

#### SECOND STAGE

Space velocity ----- Below 5 (LHSV).  
 Total pressure ----- Below 500 p.s.i.g.  
 Inlet temperature ----- Generally not substantially above about 850° F. and at temperatures minimizing cracking. 25  
 Outlet temperature ----- At least about 750° F.  
 Catalyst ----- E.g., platinum on alumina containing preferably not more than 1.0% chlorine. 30

It is to be noted that when processing the alkylate-containing feeds, lower maximum temperatures are preferred than for the alkylate free or straight run feeds because of the higher crackability of the highly branched alkylate paraffins. 35

From the defined catalytic treatment of the relatively high boiling feed stocks, not only is the paraffinic concentration substantially conserved to provide high yields of desired components for jet fuel but, as to the catalytically treated mixture that is produced, it can be subjected to a further treatment for removal of aromatics to the extent required to provide jet fuels of high luminometer number (e.g., at least 90 or more), excellent thermal stability, a high net heat value (e.g., at least about 18,850 B.t.u./lb.), a high boiling range (e.g., 350-550° F.), a low vapor pressure (e.g., maximum of about 50 p.s.i.g. at 500° F.), and other desired properties including low freeze points, the latter property being largely dependent on the iso- to normal-paraffins ratio in the charge stock. The term "iso-paraffins" as used in this discussion is meant to include all types of branched, non-cyclic paraffins irrespective of the number, location, or length of the branches. Generally speaking, the higher the ratio of iso-paraffins to normal paraffins, the lower will be the freeze point of the jet fuel product.

For the preparation of high quality jet fuels, the product mixture obtained from the catalytic dehydrogenation-isomerizing reforming treatment herein described in subjected to processing conditions selected for removal of aromatics to provide an aromatic-rich phase separate from a paraffin-rich phase comprising the desired high quality jet fuel. Thus, for example, a reduction in the aromatic concentration of the naphthene depleted product mixture can be effected by solvent extraction, as by extraction with  $\text{SO}_2$  at a liquid  $\text{SO}_2$  ratio of from about 50 to about 300 volume percent based on the product mixture, at an operating temperature of from about -20 to 50° F.

The method and process herein described provides a heretofore unknown high degree of flexibility for the production of jet fuels adapted to meet a wide variety of specific property requirements. For purposes of clearly illustrating the method of this invention, specific

embodiments are described hereinafter by the examples presented and reference to the drawings provided herewith.

FIGURE I presents curves showing a relationship between heating value and paraffin content of the jet fuel having different aromatic concentrations.

FIGURE II presents a group of curves showing a relationship of luminometer number with paraffin content of jet fuel having different aromatic concentrations.

FIGURE III presents a family of curves which establishes a relationship of equilibrium aromatic-naphthene ratios, with operating pressures and temperatures.

FIGURE IV presents a curve establishing a relationship of freeze point with concentration of high freeze point components such as n-paraffins.

The combination of conditions in terms of temperature, space velocity and hydrogen partial pressure disclosed herein were determined at least in part from a raw kerosine, derived from Barco crude, containing about 700 p.p.m. sulfur and <10 p.p.m. nitrogen which was pretreated at the conditions of 700° F., 800 p.s.i.g., 4 LHSV and 1100 s.c.f./bbl. hydrogen circulation with a cobalt molybdate on alumina catalyst whereby the sulfur concentration was reduced to 13 p.p.m. The thus-pretreated kerosine fraction boiling in the range of about 350-510° F. was then processed under a variety of operating conditions with a catalyst comprising 0.6% platinum on eta alumina and containing about 0.6% chlorine. Following such a catalytic treatment, the product mixture was distilled to remove material boiling below about 375° F. and thereafter percolated through a bed of silica gel for substantially quantitative removal of aromatics to provide highly paraffinic effluents useful as high quality jet fuels of relatively high boiling range.

In further illustration of embodiments of this invention, the following Table I sets forth data obtained by subjecting a Barco kerosine (350-510° F.), pretreated as per the aforesaid to reduce the sulfur concentration to 13 p.p.m., to the conditions shown with use of a catalyst containing 0.6% platinum on eta alumina and 0.6% chlorine.

TABLE I

| Run Numbers                                                                                                       | 1      | 2      | 3      | 4      | 5      | 6     | 7     | 8     |
|-------------------------------------------------------------------------------------------------------------------|--------|--------|--------|--------|--------|-------|-------|-------|
| (A) Treatment Conditions in Presence of Platinum Catalyst:                                                        |        |        |        |        |        |       |       |       |
| Temperature.....                                                                                                  |        |        |        |        |        |       |       |       |
| 860                                                                                                               | 900    | 860    | 800    | 650    | 750    | 940   | 900   |       |
| 500                                                                                                               | 500    | 500    | 200    | 53     | 105    | 500   | 500   |       |
| Hydrogen, partial pressure, p.s.i.....                                                                            | 455    | 445    | 445    | 180    | 48     | 95    | 450   | 455   |
| LHSV.....                                                                                                         | 20     | 45     | 60     | 30     | 10     | 20    | 15    | 3     |
| Hydrogen circulation.....                                                                                         | 6,020  | 5,010  | 5,095  | 5,535  | 5,630  | 5,875 | 5,555 | 5,940 |
| Yield, Vol. Percent, from Treatment (A):                                                                          |        |        |        |        |        |       |       |       |
| 375° F. fraction <sup>1</sup> .....                                                                               | 89.2   | 86.1   | 92.0   | 95.4   | 96.7   | 97.2  | 66.6  | 61.9  |
| 375° F. paraffins <sup>2</sup> .....                                                                              | 102    | 98     | 104    | 108    | 103    | 108   | 54    | 50    |
| Jet Fuels Produced by quantitative removal of aromatics from product from Treatment (A) by silica gel adsorption: |        |        |        |        |        |       |       |       |
| Gravity, ° API.....                                                                                               | 53.4   | 51.1   | 50.5   | 49.0   | 50.7   | 54.7  |       |       |
| Flash Point, ° F.....                                                                                             |        | 190    | 172    | 175    |        |       |       |       |
| Freeze Point, ° F.....                                                                                            | -29    | -28    | -26    | -29    | -26    |       |       |       |
| Luminometer No. ±5.....                                                                                           | 120    | 122    | 113    | 114    | 100    | 111   | 123   | 124   |
| Net Heat of Combustion (B.t.u./lb.).....                                                                          | 18,912 | 18,896 | 18,848 | 18,892 | 18,982 |       |       |       |
| Vapor Pressure (p.s.i.) at 500° F.....                                                                            | 41     | 40     | 39     |        |        |       |       |       |

<sup>1</sup> Based on 375° F. fraction in charge stock.

<sup>2</sup> Based on 375° F. paraffins in charge stock.

For the runs shown in Table I, Run Nos. 1-6, inclusive were carried out under correlated conditions selected for a high conservation of paraffins, as shown by the values of 98 to 108 volume percent shown for the yield of 375° F. paraffins from the catalytic treatment A. It is further apparent from the data in Table I that such high conservation of paraffins in such a relatively high boiling range was obtained along with a relatively high yield of the 375° F. fraction from the catalytic treatment. On the other hand, and as is evident from the data shown for Runs Nos. 7 and 8, relatively low yields were obtained for the 375° F. fraction from the catalytic treatment and paraffin retention of only about 50-54 volume percent occurred. Such results evidence the substantial loss of paraffins in the desired boiling range of at least 375° F. by use of operating conditions falling outside of the boundary limits herein defined.

In the following Table II, data are set forth for the analysis of kerosine fractions boiling in the range of about 375-500° F. from each of several different crudes. The analysis of the product obtained from a catalytic treatment thereof as embodied herein, and properties of a raffinate (jet fuel) obtained from SO<sub>2</sub> extraction of the catalytically treated product boiling in the range of about 375-500° F. are presented.

#### CONDITIONS FOR CATALYTIC TREATMENT

|                                   |         |     |
|-----------------------------------|---------|-----|
| Catalyst: platinum on eta alumina | percent | 0.6 |
| Average temperature               | ° F.    | 850 |
| Space velocity (LHSV)             |         | 20  |
| Total pressure, p.s.i.g.          |         | 450 |

TABLE II

|                                                                       | Virgin Kerosine        |                       |                            |
|-----------------------------------------------------------------------|------------------------|-----------------------|----------------------------|
|                                                                       | Mid-Continent, percent | Barco, Weight percent | West Texas, Weight percent |
| Feed Stock:                                                           |                        |                       |                            |
| Paraffins.....                                                        | 39.9                   | 42.4                  | 58.6                       |
| Naphthenes.....                                                       | 43.1                   | 43.3                  | 33.2                       |
| Aromatics.....                                                        | 17.0                   | 14.3                  | 8.2                        |
| 25 Product from Catalytic Treatment:                                  |                        |                       |                            |
| H <sub>2</sub> .....                                                  | 0.9                    | 1.0                   | 0.7                        |
| Dry Gas.....                                                          | 1.1                    | 1.6                   | 1.6                        |
| Butanes.....                                                          | 0.7                    | 1.0                   | 1.0                        |
| Pentanes.....                                                         | 0.8                    | 0.8                   | 0.8                        |
| C <sub>6</sub> -375° F.....                                           | 4.9                    | 4.8                   | 4.9                        |
| 30 375-500° F. Fraction:                                              |                        |                       |                            |
| Paraffins.....                                                        | 39.1                   | 41.0                  | 56.9                       |
| Naphthenes.....                                                       | 4.1                    | 3.7                   | 2.8                        |
| Aromatics.....                                                        | 48.4                   | 46.1                  | 31.3                       |
|                                                                       | 100.0                  | 100.0                 | 100.0                      |
| 35 Raffinate from SO <sub>2</sub> extraction of 375-500° F. fraction: |                        |                       |                            |
| Gravity.....                                                          | 52.5                   | 53                    | 54                         |
| Luminometer No.....                                                   | 110                    | 116                   | 124                        |
| Net Heat of Combustion (B.t.u./lb.).....                              | 18,920                 | 18,925                | 18,935                     |

40 It is apparent from the data set forth in Table II that by the defined catalytic reforming treatment of the 375-

500° F. boiling range kerosines, an exceptionally low make of dry gas occurred and, further, an exceptionally low overall make occurred of materials boiling below 375° F. It is further apparent from the data in Table II that the defined catalytic reforming treatment of such feed stocks resulted in substantial conservation of the paraffinic concentration in the 375° F. boiling range fraction while the naphthenes were converted in substantial amounts to aromatics.

Still other embodiments of the invention herein described are set forth in the following examples.

#### Example I

A 390 to 490° F. boiling range fraction, distilled from a West Texas crude, was pretreated over a hydrodesulphurization catalyst (chromia on alumina) at an average temperature of about 740° F., 160 p.s.i.g. total pressure,

130 p.s.i.g. hydrogen partial pressure and 0.6 LHSV whereby the sulfur concentration was reduced from about 300 p.p.m. to about 2 p.p.m. The pretreated stock thus obtained was then catalytically reformed with a 0.35% platinum on eta alumina catalyst in an adiabatic reactor system under conditions shown in the following Table III. From such a catalytic reforming treatment, liquid product in the 375° F. range was obtained in a 78.5 volume percent yield based on the amount of charge to the pretreater with a paraffin retention of at least 75.2 volume percent.

The effluent from the above catalytic reforming treatment was then distilled to obtain a 390° F. fraction which was then contacted at about 40° F. with SO<sub>2</sub> in the proportion of 200 parts SO<sub>2</sub> to 100 parts of the effluent to remove aromatics therefrom. The SO<sub>2</sub> raffinate, containing <2% aromatics, was then percolated through bauxite. The following Table III contains data for the conditions of the catalytic reforming treatment and the properties of the SO<sub>2</sub> raffinate (390° F.) following percolation through the bauxite.

TABLE III

|                                                   | First Reactor | Second Reactor | Third Reactor |  |  |  |
|---------------------------------------------------|---------------|----------------|---------------|--|--|--|
| Catalytic Treatment Conditions:                   |               |                |               |  |  |  |
| Temperature, ° F.:                                |               |                |               |  |  |  |
| Reactor Inlet.....                                | 850           | 811            | 832           |  |  |  |
| Reactor Outlet.....                               | 811           | 798            | 825           |  |  |  |
| Total pressure, p.s.i.g.....                      | 400           | 400            | 400           |  |  |  |
| H <sub>2</sub> partial pressure, p.s.i.g.....     | 330           | 330            | 330           |  |  |  |
| LHSV.....                                         | 7.6           | 2.2            | 2.2           |  |  |  |
| H <sub>2</sub> Circ., s.c.f./bbl.....             | 9,000-9,800   |                |               |  |  |  |
| Properties of 390° F. cut after Bauxite           |               |                |               |  |  |  |
| Percolation:                                      |               |                |               |  |  |  |
| Gravity, ° API.....                               | 52.7          |                |               |  |  |  |
| ASTM Dist., ° F.:                                 |               |                |               |  |  |  |
| IBP.....                                          | 400           |                |               |  |  |  |
| 10.....                                           | 410           |                |               |  |  |  |
| 20.....                                           | 414           |                |               |  |  |  |
| 50.....                                           | 424           |                |               |  |  |  |
| 90.....                                           | 458           |                |               |  |  |  |
| EP.....                                           | 493           |                |               |  |  |  |
| Luminometer No.....                               | 116           |                |               |  |  |  |
| Freeze Pt., ° F.....                              | -37           |                |               |  |  |  |
| Net Heat of Combustion, B.t.u./lb.....            | 18,938        |                |               |  |  |  |
| Flash Point, ° F.....                             | 182           |                |               |  |  |  |
| Vapor pressure at 500° F., p.s.i.g.....           | 41            |                |               |  |  |  |
| High Temp. Erdo Stability Test (300/500/600° F.): |               |                |               |  |  |  |
| Preheated Deposit Code.....                       | 1             |                |               |  |  |  |
| ΔP Hg.....                                        | 0.9           |                |               |  |  |  |

| Run No.....                                               | 1      | 2          | 3      | 4             |
|-----------------------------------------------------------|--------|------------|--------|---------------|
| Feed Stock.....                                           | Barco  | West Texas | Kuwait | Mid-Continent |
| Catalytic Treatment Conditions:                           |        |            |        |               |
| Temperature.....                                          |        |            |        |               |
| Pressure, p.s.i.g.....                                    | 862    | 862        | 860    | 860           |
| LHSV.....                                                 | 500    | 500        | 500    | 250           |
| Properties of 375° F. Jet Fuel from Silica Gel Treatment: |        |            |        |               |
| Luminometer No.....                                       | 10     | 10         | 10     | 15            |
| Net Heat of Combustion (B.t.u./lb.).....                  | 122    | 134        | 131    | 116           |
| Properties of 375° F. Jet Fuel from Silica Gel Treatment: |        |            |        |               |
| Luminometer No.....                                       | 18,960 | 18,975     | 18,975 | 18,942        |

15

20

## Example III

A West Texas raw kerosene was pretreated over a hydrodesulfurization catalyst comprising chromia on alumina promoted with molybdena at 800° F., 170 p.s.i.g., 0.8 LHSV and a hydrogen circulation rate of 695 s.c.f./bbl. The pretreated stock was then treated over a 0.35% platinum on alumina catalyst in an adiabatic reactor at the following conditions:

|    |                                             |      |
|----|---------------------------------------------|------|
| 25 | Inlet temperature, ° F.....                 | 845  |
|    | Outlet temperature, ° F.....                | 795  |
|    | Pressure, p.s.i.g.....                      | 410  |
|    | LHSV.....                                   | 7.6  |
| 30 | H <sub>2</sub> circulation, s.c.f./bbl..... | 5950 |

The product from such a treatment was distilled to obtain a 360-520° F. fraction from which aromatics were removed by silica gel absorption to produce a paraffin-rich phase having a freeze point of -28° F. By comparison, a sample of the raw kerosene percolated over silica gel to remove aromatics had a freeze point of -16° F. Data pertaining to this specific example are set forth in the following Table IV.

TABLE IV

|                                                                  | Stock                  |                                             |                                           |
|------------------------------------------------------------------|------------------------|---------------------------------------------|-------------------------------------------|
|                                                                  | Untreated Raw Kerosene | Pretreated Charge Stock (hydrodesulfurized) | Catalytically Treated (Platinum Catalyst) |
| Yield of 360° F. cut, Vol. Percent.....                          | 100                    | 94.1                                        | 93.1                                      |
| Volume yield of 360° F. paraffins.....                           | 100                    | -----                                       | 102                                       |
| Analysis of 360-520° F. Jet Fuel from above stocks: <sup>2</sup> |                        |                                             |                                           |
| Freezing Point, ° F.....                                         | -16                    | -----                                       | -28                                       |
| Paraffins, Vol. Percent.....                                     | 65.4                   | -----                                       | 84.7                                      |
| Naphthenes (monocyclic plus dicyclic).....                       | 34.5                   | -----                                       | 15.2                                      |
| Aromatic, Vol. Percent.....                                      | 0.1                    | -----                                       | 0.1                                       |

<sup>1</sup> Base.<sup>2</sup> Aromatics removed by silica gel.

## Example II

Four raw (unpretreated) kerosines (Barco, W. Texas, Kuwait and Mid-Continent) were individually treated over a 0.6% platinum on eta alumina catalyst under the following conditions and the resulting products were topped to remove materials boiling below 375° F. The 375° F. fractions were then individually percolated through silica gel whereby there were obtained paraffin-rich phases having high luminometer numbers and high net heat of combustion values.

75 A Gach Saran kerosene charge stock (boiling range 370-490° F.) was pretreated over CoMo-Al hydrodesulfurization catalyst whereby the sulfur concentration of the charge stock was reduced from 4700 p.p.m. to 8 p.p.m. and the nitrogen concentration was reduced from 80 p.p.m. to about 1 p.p.m. The pretreated charge stock was then treated over a platinum on alumina catalyst at 800° F., 370 p.s.i. (hydrogen partial pressure) and 1.5 LHSV. From such a treatment there was obtained a

## Example IV

liquid product, the 375° F. fraction of which was in 86.6 volume percent yield with a 90% volume percent conservation of paraffins.

The properties and composition of the charge stock, the catalytically treated liquid product (375° F.), and the catalytically treated product from which aromatics were removed by silica gel absorption are set forth below:

| Raw Charge Stock                      | Catalytically Treated Charge Stock |                            |
|---------------------------------------|------------------------------------|----------------------------|
|                                       | Before silica gel treatment        | After silica gel treatment |
| Composition (vol. percent):           |                                    |                            |
| Paraffins, 40.4                       | 41.9                               | 85.7                       |
| Olefins, 1.9                          | 0.6                                | (1)                        |
| Aromatics, 22.0                       | 49.4                               | (1)                        |
| Naphthenes, 35.7                      | 8.0                                | 14.3                       |
| Paraffin Distribution (vol. percent): |                                    |                            |
| C <sub>9</sub>                        |                                    | 0.8                        |
| C <sub>10</sub>                       | 1.3                                | 2.9                        |
| C <sub>11</sub> , 5.8                 | 5.7                                | 11.5                       |
| C <sub>12</sub> , 15.0                | 15.9                               | 32.8                       |
| C <sub>13</sub> , 12.4                | 12.2                               | 24.4                       |
| C <sub>14</sub> , 5.6                 | 5.2                                | 10.2                       |
| C <sub>15</sub> , 1.6                 | 1.6                                | 2.5                        |
| C <sub>16</sub>                       |                                    | 0.6                        |
| Distillation (ASTM):                  |                                    |                            |
| IBP, 371                              | 392                                |                            |
| 5%, 399                               | 407                                |                            |
| 10%, 405                              | 410                                |                            |
| 20%, 412                              | 414                                |                            |
| 50%, 427                              | 432                                |                            |
| 90%, 457                              | 477                                |                            |
| EP, 499                               | 498                                |                            |
| Luminometer No.                       | 114                                |                            |
| Freeze point, ° F.                    | 45                                 |                            |
| Heating Value (B.t.u./lb.)            | 18,920                             |                            |

<sup>1</sup> Nil.

### Example V

A 368 to 473° F. boiling range fraction, distilled from a Barco virgin kerosene, was pretreated with a cobalt molybdate hydrodesulfurization catalyst at 700° F., 800 p.s.i.g. hydrogen pressure and 4.0 LHSV whereby the fraction was reduced in nitrogen concentration to 2 p.p.m. and sulfur to 6 p.p.m. The pretreated fraction was then treated over a 0.6% platinum on eta alumina catalyst at 900° F., 10 LHSV, 250 p.s.i.g. pressure and a ratio of H<sub>2</sub>/feed of 20 (mol:mol). Such a treatment resulted in substantial conversion of naphthenes in the feed stock to aromatics with a paraffin retention of about 70%. By extraction of aromatics from the thus-treated product mixture by silica gel, a paraffin-rich raffinate was obtained that had a luminometer number of >120.

In reference to the jet fuels produced by the method of this invention, and in the defined high yields from the relatively high boiling feed stocks as described hereinbefore, the following is a typical analysis (mass spectrographic) of a jet fuel produced by the process embodied herein from a West Texas kerosene having a boiling range of from about 390 to about 490° F. by treatment over a 0.35% platinum on eta alumina catalyst followed by substantial but not complete removal of aromatics by SO<sub>2</sub> absorption. Such a jet fuel consists essentially of C<sub>11</sub> to C<sub>16</sub> paraffins, naphthenes and not more than 5 vol. percent aromatics.

### CARBON NO. DISTRIBUTION, VOL. PERCENT

| Paraffins:      | 10.8 |
|-----------------|------|
| C <sub>11</sub> | 30.4 |
| C <sub>12</sub> | 30.0 |
| C <sub>13</sub> | 9.9  |
| C <sub>14</sub> | 2.4  |
| C <sub>15</sub> | 2.7  |
| C <sub>16</sub> | 0.3  |
| C <sub>17</sub> | 0.2  |
| C <sub>18</sub> | 0.2  |
| C <sub>19</sub> | 7.6  |
| Naphthenes      | 4.9  |
| Aromatics       | 0.6  |
| Misc.           |      |

A typical analysis of a jet fuel, prepared in the manner

5

of the jet fuel for which the foregoing analysis is set forth, except that the feed stock had an initial boiling point of about 375° F. and aromatics were substantially quantitatively removed by silica gel adsorption, is as follows:

Luminometer No. ----- >112  
Net heat of combustion B.t.u./lb. ----- >18,900

### CARBON NO. DISTRIBUTION (MOL. PERCENT)

#### Paraffins:

|    |                       |      |
|----|-----------------------|------|
| 10 | C <sub>10</sub> ----- | 2.9  |
|    | C <sub>11</sub> ----- | 17.4 |
|    | C <sub>12</sub> ----- | 12.2 |
|    | C <sub>13</sub> ----- | 13.3 |
|    | C <sub>14</sub> ----- | 11.5 |
|    | C <sub>15</sub> ----- | 15.4 |
|    | C <sub>16</sub> ----- | 12.8 |
|    | C <sub>17</sub> ----- | 4.3  |
|    | C <sub>18</sub> ----- | 0.7  |
| 15 | Naphthenes -----      | 9.4  |
| 20 | Aromatics -----       | 0.1  |

As shown, and although such a product contains a small amount of C<sub>10</sub> paraffins and C<sub>18</sub> paraffins, it consists essentially of paraffins in the C<sub>11</sub> to C<sub>16</sub> range and naphthenes. Thus, in general, the jet fuels embodied herein are substantially composed with respect to paraffins to those of C<sub>11</sub> and higher carbon atom-containing paraffins and may or may not contain some C<sub>10</sub> paraffins. When present, however, the C<sub>10</sub> paraffins do not usually exceed about 5 volume percent. Such jet fuels are further characterized by being devoid of or substantially devoid of C<sub>9</sub> and lower paraffins. However, if C<sub>9</sub> paraffins are present, they are present in relatively small amount (e.g., not more than 2% and more specifically not more than about 1%) which may be due to phase equilibrium in carryover in a distillation operation employed in the process. In general, the jet fuels embodied herein have a net heat of combustion of at least about 18,800 b.t.u./lb. and comprise a mixture of paraffins, naphthenes and aromatics in which the aromatics concentration is less than 10 volume percent and usually less than about 5 volume percent.

### Example VI

The catalytically treated and silica gel extracted product of Example IV above presented was given a subsequent treatment over a 0.35% platinum on alumina catalyst under isomerization conditions of:

Temperature, ° F. ----- 800  
Pressure, p.s.i.g. ----- 350  
LHSV, v./v./hr. ----- 1

This further isomerization step significantly lowered the n-paraffin content, and thus the freeze point. Under these conditions, additional dehydrogenation of retained naphthenes was also experienced. The results of this specific example are shown in the following table:

|                                | Feed to Isomerization Step | As Produced | After Removal of Aromatics With Silica Gel |
|--------------------------------|----------------------------|-------------|--------------------------------------------|
| Paraffins, percent vol.        | 84.7                       | 84.3        | 96.7                                       |
| Olefins, percent vol.          | 0.7                        | 0.7         | 0.3                                        |
| Naphthenes, percent vol.       | 15.2                       | 2.2         | 2.5                                        |
| Aromatics, percent vol.        | 0.1                        | 12.8        | 0.5                                        |
| Freeze Point, ° F.             | -28                        | -74         | -68                                        |
| Normal Paraffins, percent vol. | 34                         | 7.4         | 8.5                                        |

### Example VII

The kinetics of three reactions of prime interest (naphthalene dehydrogenation, isomerization of normal paraffins, and paraffin hydrocracking) were obtained under catalytic reforming treatment of a hydrodesulfurized West Texas kerosene passed in contact with a fresh catalyst comprised of 0.6% platinum on eta alumina. Using reciprocal LHSV (units of v./v./hr. or just hr.<sup>-1</sup>)

60

65

70

75

as a measure of time in the rate constant,  $k$ , the following values were obtained:

| Reaction                          | Naphthene Dehydrogenation | Isomerization | Paraffin Hydro-cracking |
|-----------------------------------|---------------------------|---------------|-------------------------|
| $k$ 850° F., hr. <sup>-1</sup>    | 60                        | 2.8           | 0.36                    |
| Activation Energy, Kcal./gr. mol. | 30                        | 41            | 57                      |

From these results, it is evident that the dehydrogenation reaction proceeds most rapidly and that isomerization requires much lower space velocity (higher residence time) or higher temperature. Furthermore, the relatively high activation energy for the undesirable hydrocracking reaction teaches us that for any level of isomerization desired, the lower the temperature at which this is conducted, the less is the paraffin cracking and the greater the paraffin retention.

#### Example VIII

In order to show that use of conditions of high temperature without sufficiently high space velocity result in a very substantial loss of paraffins in the desired boiling ranges, the following data are set forth for runs using 0.6% platinum on alumina catalyst with a 350-510° F. boiling range Barco kerosene pretreated to a sulfur concentration of about 13 p.p.m.

|                                                          | Untreated Charge Stock | Run No. |
|----------------------------------------------------------|------------------------|---------|
|                                                          | 1                      | 2       |
| <b>Reaction Conditions:</b>                              |                        |         |
| Temperature, ° F.                                        | 942                    | 940     |
| Pressure, p.s.i.g.                                       | 500                    | 500     |
| LHSV                                                     | 3                      | 5       |
| H <sub>2</sub> Circulation, s.c.f./bbl.                  | 7,170                  | 4,866   |
| <b>Yields:</b>                                           |                        |         |
| Dry Gas (wt. percent)                                    | 10.9                   | 6.7     |
| Butanes (vol. percent)                                   | 7.1                    | 4.7     |
| Pentanes (vol. percent)                                  | 4.9                    | 5.6     |
| C <sub>6</sub> -375° F. (vol. percent)                   | 16.4                   | 43.0    |
| 375° F. cut (vol. percent)                               | 83.6                   | 33.2    |
| <b>Composition of 375° F. cut vol. percent, on feed:</b> |                        |         |
| Paraffins                                                | 37.7                   | 4.2     |
| Naphthenes                                               | 35.1                   | 0.2     |
| Aromatics                                                | 10.8                   | 28.8    |
| Retention of 375° F. Paraffins, vol. percent             | 100                    | 11      |
|                                                          |                        | 24      |

As shown by such data, and as compared to the paraffin concentration in the 375° F. fraction of the feed stock, a paraffin retention of only 11 and 24 volume percent, respectively, occurred for the runs carried out at relatively high temperatures but without use of a substantially high space velocity.

In the use of acid extraction (e.g., oleum) for aromatic-removal, it may often be necessary to further treat the extracted product to effect additional removal of aromatics. For such a purpose, a suitable method involves subjecting the paraffin-rich phase from the acid extraction to hydrogenation for conversion of the remaining small amount of aromatics to naphthenes. A suitable combination of conditions for such a treatment is as follows:

Pressure, p.s.i.g. (total) 500 or higher.  
Space velocity LHSV 1.  
H<sub>2</sub>/charge hydrocarbons (mol ratio) 16 (approx.).  
H<sub>2</sub>/charge hydrocarbons (s.c.f./bbl.) 10,000.  
Temperature, ° F. 500.

Catalyst: hydrogenation catalyst e.g., platinum on cta or gamma alumina

As used herein, luminometer number is determined in accordance with the method of test, set forth in ASTM Description D1740-60T.

It will be apparent to those skilled in the art, that in a process as herein described for the production of jet fuels of defined boiling range, as for example, an initial boiling point of at least 350° F., or at least 375° F., that any lower boiling material that may be formed during the process may be removed by conventional means, such as by distillation, in any of several stages of the process. Removal of such low boiling materials may be carried

out by subjecting the product, from the catalytic reforming step for conversion of naphthenes to aromatics or after the second catalytic isomerizing step, to distillation to strip out the undesired materials that boil below the initial boiling point of the desired jet fuel.

In certain instances freeze point depressants may be added to lower the freeze point and, for this purpose, isoparaffins such as alkylates that boil within the boiling range of the jet fuel can be used. The addition of isoparaffins for lowering the freeze point can be made to the feed stock, to the jet fuel product or to an intermediate stage of the process herein described.

In the present process, use of an adsorbent such as silica gel for aromatic removal usually does not require further processing of the product jet fuel as the paraffin rich effluent therefrom is generally of exceptionally desirable characteristics with respect to luminometer number and thermal stability. Similarly, in the use of SO<sub>2</sub> for aromatic removal, further processing of the raffinate from such an operation is generally not required. However, a further treatment of the SO<sub>2</sub> raffinate, such as with an adsorbent clay, or catalytic hydrogenation may be used to improve thermal stability by removal of residual contaminants that tend to decrease thermal stability.

Referring now to FIGURE I, the data obtained in this investigation were accumulated and developed to produce the self-explanatory curves presented in the figure which show the change in heating value of jet fuels as their paraffin and aromatic content is varied. The curves in FIGURE I (and FIGURES II-IV) were established for fuels having a nominal boiling range of 350-500° F. For fuels of significantly different boiling ranges, the curves would be similar but displaced with respect to the abscissus. FIGURE II, on the other hand, shows the variation in luminometer number obtained as the paraffin content varies for three different aromatic products. The figure is essentially self-explanatory in showing that a higher LN is obtainable as the aromatics are reduced in the product and the higher the paraffin content, the higher will be the (LN) luminometer number.

FIGURE III presents an accumulation of data arranged to provide a family of curves which permit establishing a relationship between equilibrium aromatic-naphthene ratio, hydrogen pressure and temperature of the reforming operation to effect the desired change in composition to produce a desired jet fuel product. The relationships established by the curves presented in FIGURE III show that to obtain a given aromatic/naphthene ratio, different hydrogen pressure conditions are required for different reaction temperature conditions.

FIGURE IV entitled Effect of n-Paraffin Concentration on Freeze Point for 375-500° F. Boiling Kerosene Fraction shows a single straight line curve which establishes a relationship between concentration of n-paraffins in the product and the freeze point of the product. This relationship is particularly useful in identifying the process requirements for producing a jet fuel for the reasons more fully explained below.

In accordance with one specific embodiment of this invention the curves above-identified are employed in the following illustration to identify the procedure for producing a desired 100LN jet fuel boiling in the range of from about 350° F. to about 500° F. and having for example, a freeze point of about -40° F. and a heating value of about 18,900 B.t.u./lb. From FIGURE 1, we determine that a jet fuel of about 18,900 B.t.u./lb. heating value must have a paraffin content of at least 85% if there is as much as 2% of aromatics in the jet fuel product. From FIGURE II, we also determine that to produce a product having an LN of 100 that the product must have at least about 82% paraffins when as much as 2% aromatics is in the product. Therefore, from these two figures we now know that a jet fuel product of at least 85% will be suitable to produce a 100+ LN product hav-

ing a heating value of 18,900 B.t.u./lb. Turning now to FIGURE IV we determine that the jet fuel product suitable to meet a -40° F. freeze point should not have substantially greater than about 23 volume percent of normal paraffins. That is, the sum of the concentrations of low freeze point constituents such as isoparaffins must be at least about 77 volume percent so that when combined with the n-paraffin material, the final product will meet the -40° F. freeze point requirement. However, from FIGURES I and II we determined that the paraffin concentration of the final product must be at least 85% and since only about 23 volume percent of this can be n-paraffins, it is thus essentially that about 62% of the paraffins must be iso-paraffins to meet the product requirements.

In the method and process of this invention, the iso-paraffin concentration requirement may be obtained by one or more different routes which include: (1) isomerizing n-paraffins in the feed, (2) blending isoparaffin alkylate product with the dehydrogenated product obtained as above described or (3) a combination of (1) and (2) above. By the above discussion we have been able to identify the requirements of the product components with the aid of FIGURES I, II and IV.

To produce the product thus identified, applicants have found and identified a relationship of operating condition that when properly correlated will produce the product desired. Accordingly, a further embodiment of this invention is directed to identify the method and operating procedure one employs for producing a product such as above-identified.

As an initial step of the process, the composition of the kerosene feed with respect to paraffins, naphthenes and aromatics must be determined. Having thus made this determination and identified the characteristics of the product required we determine from FIGURE I the paraffin-naphthene ratio permissible in the final product having about 2% aromatics therein. From FIGURE I we determine the naphthene concentration to be about 13% and thus, the paraffin/naphthene ratio to be 85/13 or about 6.5.

As indicated above, the kerosene feed to be processed is evaluated to determine its paraffin, naphthene and aromatic content. Assuming that we determine that the feed comprises 40% paraffins we can determine from the above paraffin-naphthene ratio to what extent the naphthenes in the feed must be reduced to produce the 6.5 ratio above determined. With 40% paraffins in the feed we find by the above relationship that the naphthene content must be reduced to about 6.1%. This determination also establishes the aromatic content of the product after the catalytic treatment and before aromatic extraction, as about 53.9 and therefore the aromatic/naphthene ratio as 53.9/6.1 or about 8.9 as a minimum value. Having thus determined to what extent the feed needs to be reformed by dehydration of naphthenes to produce a product having an aromatic/naphthene ratio of about 8.9 we now determine from FIGURE III the pressure-temperature relationship required to produce such a product. It will be observed from FIGURE III that the correlated operating conditions to produce the above aromatic/naphthene ratio are as follows:

| At, ° F.: | H <sub>2</sub> pressure must not be more than about p.s.i.a. |
|-----------|--------------------------------------------------------------|
| 750       | 200                                                          |
| 775       | 270                                                          |
| 800       | 350                                                          |
| 825       | 450                                                          |

In accordance with the correlations shown in FIGURE 4 it can be determined that to obtain the desired -40° F. freeze point of this example, that the n-paraffin content should be no more than about 23% in the product fuel or 27% of the paraffin fraction. Referring thus to our example for a raw, untreated feed containing 40% total

5 paraffins, if the n-paraffin content is thus more than about 27% x 40% or about 10.8% normal paraffins, isomerization of the feed will be required under the conditions hereinbefore set forth. It is obvious that the greater the concentration of normal paraffins in the feed, the greater will be the amount of isomerization required.

Having thus provided a general description of the invention and presented several examples in support thereof, it is to be understood that no undue limitations are to be imposed by reason thereof except as defined by the following claims.

We claim:

1. A method for producing jet fuels of desired freeze point and heating value which comprises: determining from the correlation represented by FIGURE IV the permissible n-paraffin content of a kerosine boiling range hydrocarbon to provide a product of desired freeze point; determining from the correlations represented by FIGURES I and II the maximum concentrations of naphthenes and/or aromatics permissible in the finished jet fuel product to maintain as a minimum a predetermined heating value and luminometer number desired, having thus determined the paraffin-naphthene-aromatic product distribution, determining the aromatic/naphthene ratio required in the effluent of a catalytic dehydrogenation-isomerization step and then catalytically reforming a paraffin rich kerosine boiling range feed in accordance with the relationship of conditions provided in the equilibrium correlation represented by FIGURE III for the above determined aromatic/naphthenic ratio at a space velocity chosen to retain at least about 70% of the paraffins and removing aromatics from the reformed effluent to provide the product distribution above determined.

2. The method of claim 1 wherein the dehydrogenation of the hydrocarbon feed is accompanied with isomerization of n-paraffins in an amount sufficient to provide the product with a desired freeze point, the degree of isomerization required being determined by the freeze point correlation represented by FIGURE IV.

3. The method of claim 1 wherein the first catalytic treatment is primarily dehydrogenation of naphthenes and wherein isomerization of paraffin hydrocarbons is accomplished in a downstream stage of catalytic treatment at suitably correlated temperature and space velocity conditions, and the extent of isomerization effected being sufficiently severe such that the normal paraffins are reduced to below about 30% of the total paraffin content.

4. A method for producing a kerosine boiling range jet fuel having a freeze point below about -40° F. and a B.t.u./lb. heating value in excess of 18,900 which comprises: determining from FIGURE IV the maximum permissible amount of n-paraffin allowed in the product to meet said freeze point requirements, determining from correlations represented in FIGURES I and II the permissible paraffin-naphthene-aromatic content to satisfy desired product requirements of heating value and a luminometer number of at least 90, having thus made the above determinations, determining the required naphthene to aromatic ratio in the product effluent of a catalytic dehydrogenation-isomerization conversion of the kerosine boiling feed, thereafter catalytically dehydrogenating naphthenes in said feed in accordance with the temperature and pressure correlation of FIGURE III to obtain said required product effluent naphthene to aromatic ratio, maintaining isomerizing conditions in a least one downstream stage of said catalytic treatment to permit obtaining the above determined n-paraffin limit employing a space velocity in each of said dehydrogenating and isomerizing operations to retain at least about 70% of the paraffins and removing aromatics from the product of said catalytic treatment to produce the above determined permissible paraffin-naphthene-aromatic content of said product.

5. The method of claim 4 wherein alkylate product boiling in the kerosine boiling range is employed with the

kerosine boiling feed to provide the jet fuel product desired.

6. The method of claim 1 wherein sufficient alkylate is blended with the product of the catalytic dehydrogenation step to produce the desired jet fuel product.

References Cited

UNITED STATES PATENTS

3,110,661 11/1963 Franz ----- 208—60  
3,117,073 1/1964 Hertwig et al. ----- 208—65 10

FOREIGN PATENTS

870,474 6/1961 Great Britain.

OTHER REFERENCES

- Popovich et al., Fuels, Lubricants (1959), pp. 156—163, John Wiley and Sons.  
5 Paushkin, The Chemical Composition and Properties of Fuels for Jet Propulsion (Chapter II, part 4), pp. 53—64 (1962), Pergamon Press.

HERBERT LEVINE, *Primary Examiner.*